

## UNITED STATES PATENT OFFICE

2,111,470

PROCESS FOR ELECTROLYTIC PREPARA-  
TION OF ALKALINE-EARTH ALLOYS

Robert André Gadeau, Saint Jean De Maurienne, France, assignor to Compagnie de Produits Chimiques et Electrometallurgiques Alais, Fruges et Camargue, Paris, France, a corporation of France

No Drawing. Application April 18, 1936, Serial No. 75,240. In Germany May 27, 1935

3 Claims. (Cl. 204—19)

Up to the present day, calcium has been prepared exclusively by electrolysis of its molten chloride; by reason of the difficulty of the preparation of anhydrous calcium chloride and the 5 special difficulties in the electrolysis, calcium is still a very expensive metal.

It has already been proposed a long time ago, to subject to electrolysis various molten chlorides which contain the corresponding oxide in solution. The process appears valuable for the preparation of cerium, but it could never be applied for the preparation of the alkaline earth metals. My experiments have shown that the electrolysis of a molten bath of calcium chloride, which contains dissolved lime, leads at once to the formation of a thick slime, which makes the electrolysis as good as impossible. Moreover it is known that the basic chlorides of calcium dissolve metallic calcium, whereby slimy masses are 20 formed and the resistance of the bath is increased.

Since the decomposition voltages of calcium oxide and calcium chloride lie close to one another, there takes place, in a molten bath of these two compounds, always in part an electrolysis of the chloride, even if the bath is saturated with lime, which manifests itself in a troublesome evolution of chlorine and a costly consumption of chloride.

I have found, and this is the essential characteristic of the present invention, that all these difficulties are avoided and that it is possible easily to obtain alkaline earth metals by electrolysis of their oxides, provided that an alkaline earth chloro-fluoride is utilized as oxide-dissolving electrolyte.

My experiments have shown that in an electrolyte, of which the composition corresponds for example to the formula  $\text{CaCl}_2 \cdot \text{CaF}_2$ , the properties of calcium chloride are so far concealed, 40 that no appreciable volatilization of the bath takes place at about  $800^\circ$ , the chloride no longer takes part in the electrolysis and the bath no longer dissolves any appreciable quantity of metallic calcium, whereby the formation of a 45 slime of basic salts is suppressed.

The process according to the invention is particularly applicable to the manufacture of alloys of the alkaline earth metals with heavy metals like lead, copper, zinc, etc. A bath with bottom 50 made of carbon and walls made of carbon or refractory material contains at the bottom the molten heavy metal, which forms the cathode; the anode is a carbon rod which dips into the electrolyte consisting of alkaline earth chloro-fluoride, to which from time to time alkaline earth

oxide is added. The oxide becomes electrolyzed; the alkaline earth metal alloys itself with the heavy metal of the cathode, the oxygen burns away the anode, with evolution of carbon monoxide.

A suitable electrolyte for the preparation of calcium is calcium chloro-fluoride  $\text{CaCl}_2 \cdot \text{CaF}_2$ , i. e., a mixture of approximately 60 percent by weight of calcium chloride and 40 percent by weight of calcium fluoride, in which lime is dissolved. The invention however is not limited to that composition; there is no objection to adding an excess of calcium fluoride. The only limitation is by the rise of the melting point of the mixture, which is at  $950^\circ$  with 50 percent by weight 10 of calcium fluoride. One may also be satisfied with a lower content of calcium fluoride; I have indeed ascertained that calcium chloride was already stabilized substantially by 10 to 20 percent by weight of calcium fluoride. While lime is 15 added periodically, the molten bath is electrolyzed at 6 to 8 volts tension between carbon anodes and a cathode layer of molten lead, which is disposed at the bottom of the bath, wherein the working temperature amounts to about  $800^\circ$ . In 20 this way there is obtained, with a current yield 25 of 50 percent, a lead-calcium alloy, in which the calcium is extremely cheap, and which can be utilized as it is for numerous applications.

It is to be quite understood that the invention 30 is not limited to the example mentioned; in the same way there can be produced various other alloys other than lead-calcium, for example zinc-calcium, copper-calcium and so on.

The process is also applicable under the same 35 conditions to the preparation of alloys of barium and of strontium.

Lastly, it is possible to maintain the electrolysis not with an alkaline earth oxide, but with a compound which forms the oxide under the influence of heat, for example with a carbonate, 40 oxalate, acetate, and so on. In particular it is of advantage, for example, to prepare calcium from calcium carbonate, consequently an extremely cheap mineral.

I have found that pure calcium can be easily prepared by electrolytic refining of its heavy alloys which have been obtained according to the present invention. For this the same electrolyte is very well suited; the poles of the bath can 50 therefore be reversed and the carbon electrode replaced for example by a cooled iron cathode, upon which a tube of calcium is then obtained.

I have found further that by electrolytic refining of the heavy alloys, prepared according to the 55

present invention, also alloys of aluminium and magnesium with calcium can be easily prepared. It suffices to reverse the poles of the bath and to dispose on the surface of the bath a molten cathode layer of aluminium or magnesium, into which the current is led by a carbon electrode. Electrolysis at a voltage of a few volts causes the calcium of the heavy alloy at the anode to pass into the light alloy at the cathode, with a current yield of approximately 100 percent. In the foregoing description and in the claims, there should be understood by the term "alkaline earth metals" calcium, barium and strontium, to the exclusion of magnesium, the properties of the last differing entirely, from the point of view of electrolysis and the point of view of chemistry from those of calcium, barium and strontium.

What I claim is:

1. A method of manufacturing an alloy of an alkaline earth metal of the group consisting of calcium, barium and strontium with a heavy metal of the group consisting of lead, zinc and copper, by electrolysis with a carbon anode and a cathode consisting of said fused heavy metal, which comprises dissolving an oxide of said alkaline earth metal in a fused chloro-fluoride of said
- 20
- 25

alkaline earth metal, and electrolyzing the fused bath thus obtained.

2. A method of manufacturing an alloy of an alkaline earth metal of the group consisting of calcium, barium and strontium with a heavy metal of the group consisting of lead, zinc and copper, by electrolysis with a carbon anode and a cathode consisting of said heavy metal in the fused state, which comprises dissolving a carbonate of said alkaline earth metal in a fused 5 10 chloro-fluoride of said alkaline earth metal, to give off by the heat of said chloro-fluoride the oxide of said alkaline earth metal, and electrolyzing the fused bath thus obtained.

3. A method of manufacturing an alloy of an alkaline earth metal of the group consisting of calcium, barium and strontium with a heavy metal of the group consisting of zinc, lead and copper, by electrolysis with a carbon anode and a cathode consisting of said heavy metal in the 15 20 fused state, which comprises dissolving lime in a mixture of from 90 to 40 per cent in weight of fused calcium chloride and from 10 to 60 per cent in weight of fused calcium fluoride, and electrolyzing the fused bath thus obtained. 25

ROBERT ANDRÉ GADEAU.